

T. B. PARKISON.

PROCESS OF MANUFACTURING MINERAL WOOL.

APPLICATION FILED NOV. 10, 1908.

945,583.

Patented Jan. 4, 1910.



# UNITED STATES PATENT OFFICE.

THOMAS BRADY PARKISON, OF MUNCIE, INDIANA, ASSIGNOR TO UNION FIBRE COMPANY, OF WINONA, MINNESOTA, A CORPORATION OF MINNESOTA.

## PROCESS OF MANUFACTURING MINERAL WOOL.

945,583.

Specification of Letters Patent. Patented Jan. 4, 1910.

Application filed November 10, 1908. Serial No. 461,943.

To all whom it may concern:

Be it known that I, THOMAS B. PARKISON, a citizen of the United States, residing at Muncie, in the county of Delaware and State of Indiana, have invented a new and useful 5 Process of Manufacturing Mineral Wool, of which the following is a specification.

My invention relates to a process of manufacturing mineral wool, the same being an 10 improvement on the process described in Patent, No. 779,307, granted to me on the third day of January, 1905, wherein the molten slag or scoria as it comes from the cupola is forced into a blow tube, and is 15 then brought into intimate contact with hot vapors and smoke from a furnace, which commingling of the smoke and the hot filamentous slag acts to elongate, soften and toughen the fibers of the mineral wool and 20 completely convert the slag into filaments, the slag being otherwise only partially converted and being partially solidified into the form of beads.

The object of the present invention is to 25 render water-proof the mineral wool formed in the manner described, by coating the fibers or filaments of the wool with a thin layer of oil, thus not only water-proofing the fiber, but rendering the fibers of the 30 mineral wool more adhesive and clinging so that when they are finally felted or intermingled with the fibers of flax, paper stock, etc., as described in Patents Nos. 811,227, 683,208, and 688,420, and in my 35 pending application Serial No. 510,670, filed July 31, 1909, to form insulating boards or blocks, the material so formed will have a closer consistency and greater cohesion than when not so previously coated with oil.

40 A further object is to not only water-proof and render the fibers adhesive, as already described, but also to soften and anneal the fibers, materially lengthen them, and give extra tensile strength thereto by 45 subjecting them in their passage from the steam blast to the blow tube to the smoke of vaporized hydrocarbon, thus accomplishing the water-proofing and annealing in one operation, and intimately intermingling the 50 hydrocarbon with the fiber.

The mineral wool treated as above described, is particularly applicable for use in the process for forming insulating boards and blocks described in my pending application above referred to, but I do not wish

to be limited to this application of my invention, as the water-proofed fibers may be used for any purpose to which they are applicable without departing from the spirit thereof. 60

In the accompanying drawings:—Figure 1 is a side elevation of an apparatus whereby my improved process may be carried into effect. Fig. 2 is a detail section of the petroleum or other hydrocarbon sprinkler or distributor. 65

Similar reference numerals designate corresponding parts in all the figures of the drawings.

In the drawings, 1 designates a cupola 70 furnace of any ordinary or available type, 2 the slag outlet, and 3 a blast nozzle opening slightly below the outlet 2, the air or steam blast from which projects the stream of molten slag through a blow tube or cylinder 4 into a settling chamber, not shown. 75

The elements above described are well known in the process of making mineral wool, but in addition thereto, I provide means whereby the smoke from a heavy 80 crude hydrocarbon oil, such as crude petroleum or like hydrocarbon products, shall be intimately projected into and permeate the mass of molten or incandescent fibers as they are blown through the blow tube 4; 85 and I also preferably provide means whereby the hydrocarbon oil shall be brought into contact with the molten slag or scoria while still in a highly heated condition, thus vaporizing the oil, the residue or smoke of the 90 vaporized hydrocarbon being thus brought into intimate contact with the exterior surfaces of the flying filaments of molten slag and thoroughly coating the same. In order 95 to attain this step of my process, I may use various means, but I illustrate for this purpose a pipe 5 leading from a tank 6 provided with a supply pipe 7, and containing petroleum or other preferably heavy, crude hydrocarbons. The lower end of the pipe 6 is provided with any suitable means of distributing the oil in small streams or drops upon the jet of molten slag, such as the perforated pipe or tee 8 illustrated in detail 100 in Fig. 2, wherein the dotted circles indicate 105 the jet.

It will be seen that by introducing the oil into the molten slag prior to its entrance into the blow tube and while it is in flight or transit, the oily smoke generated by the in- 110

candescent slag through the combustion of the oil will be inclosed within the blow tube, and will therefore more completely impregnate the mass of filamentous material.

- 5 While the vaporizing and carbonizing of the oil by means of the molten or incandescent slag is desirable, I do not wish to be limited to this, as it is within my invention to generate this hydrocarbon vapor and to
- 10 produce carbonization of the vapor in any other manner desired and to bring this carbonized vapor into contact with the blast of slag while in flight or transit at any point between the opening of the cupola and the exit of the slag through the blow tube. It is also to be understood that any form of apparatus may be employed for carrying out this process suitable for the purpose; that by the term "slag", is intended to embrace any substance or material from which mineral or rock wool is or may be produced; and that while the mineral wool produced by the process above described is referred to as being particularly applicable for use
- 15 20 25 30 in making insulating blocks, boards etc., as described in my pending application, I do not of course wish to be limited to this application of the product, but reserve the right to modify or vary the described process or its application at will within the scope of the protection prayed.

Having thus fully described my invention, what I claim as new, and desire to secure by Letters Patent, is:—

- 35 1. A process for the production of water-proof mineral wool, which consists in projecting a blast of molten slag in the form of highly heated filaments and subjecting the same to the action of oil whereby each 40 individual filament is coated therewith.
2. A process for the production of water-proof mineral wool, which consists in projecting molten slag in the form of highly heated filaments, and subjecting said fila-

ments while being so projected and while so 45 heated to the action of a liquid hydrocarbon.

3. A process for the production of water-proof mineral wool, which consists in subjecting a blast of molten slag while in transit 50 to the action of vaporized hydrocarbon oil and smoke generated by the contact of said oil with a blast of molten slag.

4. A process for the production of water-proof mineral wool, which consists in bringing finely divided hydrocarbon oil into contact with a projected blast of filamentous slag, atomizing the oil by the blast, and burning the atomized oil by contact with the molten filaments.

5. A process for the production of water-proof mineral wool, which consists in projecting a blast of hot slag or scoria, and bringing it into direct contact with the oil.

6. A process for the production of water-proof mineral wool, which consists in projecting a blast of hot slag or scoria and subjecting the projected material in transit to the action of smoke from burning oil in front of said blast, whereby each individual 70 filament is coated with oil.

7. A process for the production of water-proof mineral wool, which consists in projecting the hot slag or scoria, and spraying a liquid hydrocarbon thereon while in 75 transit.

8. A process for the production of water-proof mineral wool, which consists in projecting the molten slag or scoria by a blast, and spraying liquid hydrocarbon thereon 80 immediately in front of said blast.

In testimony, that I claim the foregoing as my own, I have hereto affixed my signature in the presence of two witnesses.

THOMAS BRADY PARKISON.

Witnesses:

WILLIAM M. OVERMIRE,

LULA B. ADAMS.